

## [54] METHOD AND APPARATUS FOR COLD-DRAWING METALLIC TUBES

[75] Inventors: **Helmut Benteler**, Bielefeld; **Franz-Josef Hartmann**, Paderborn; **Heinz Hefendehl**, Schloss Neuhaus, all of Germany

[73] Assignee: **Benteler-Werke AG**, Schloss Neuhaus, Kreis Paderborn, Germany

[22] Filed: **June 26, 1972**

[21] Appl. No.: **265,970**

## [30] Foreign Application Priority Data

June 24, 1971 Germany ..... 2131343

[52] U.S. Cl. .... **72/43, 72/60, 72/283**

[51] Int. Cl. .... **B21c 3/14**

[58] Field of Search ..... **72/43, 42, 45, 283, 60**

## [56] References Cited

## UNITED STATES PATENTS

|           |         |                      |        |
|-----------|---------|----------------------|--------|
| 2,308,120 | 1/1943  | Staples et al.....   | 72/283 |
| 2,351,710 | 6/1944  | Sanders.....         | 72/283 |
| 3,292,407 | 12/1966 | Poncar.....          | 72/283 |
| 3,526,115 | 9/1970  | Armstrong et al..... | 72/45  |
| 2,173,099 | 9/1939  | Dennis.....          | 72/283 |
| 2,355,734 | 8/1944  | Katz.....            | 72/283 |

## FOREIGN PATENTS OR APPLICATIONS

571,905 3/1959 Canada ..... 72/271

## OTHER PUBLICATIONS

"Promotion of Fluid Lubrication in Wire Drawing";

by Christopherson et al.; pp. 643-653; Pro. Inst. Mech. Eng., 1955, Vol. 169.

Primary Examiner—Richard J. Herbst  
Attorney, Agent, or Firm—Michael S. Striker

## [57] ABSTRACT

Steel tubes are cold-drawn in a bench wherein the reducing die is located in front of a sleeve defining with the external surface of the tube to be cold-drawn an elongated tubular confining space which tapers toward the die at an angle of less than 3°. The space is filled with a lubricant at an elevated pressure of up to 100 atmospheres superatmospheric pressure, and such pressure rises automatically to a value exceeding at least 10 times the initial pressure when the tube is moved lengthwise at a speed of up to and in excess of 300 meters per minute. The rise in pressure of confined lubricant is due in part to friction between the lubricant and the external surface of the tube and suffices to insure that the moving tube remains out of mechanical contact with the die. A similar forwardly tapering confining space for reception of a pressurized lubricant can be provided between the internal surface of the tube and a confining member which is connected to and located behind a floating mandrel. The thus treated tube can be subjected to one or more additional cold-drawing treatments to reduce its outer diameter from 8-35 millimeters to about 3 millimeters and its wall thickness from about 3.5 millimeters to about 1 millimeter.

25 Claims, 2 Drawing Figures





PATENTED MAR 26 1974

3,798,943

SHEET 2 OF 2



FIG. 2

## METHOD AND APPARATUS FOR COLD-DRAWING METALLIC TUBES

### BACKGROUND OF THE INVENTION

The present invention relates to a method and apparatus for cold-drawing metallic tubes or billets, especially steel tubes. More particularly, the invention relates to improvements in a method and apparatus for cold-drawing tubes or billets (hereinafter called tubes) in a draw bench wherein the surfaces of the tubes are separated from internal and/or external diameter- and/or wall thickness-reducing devices by layers or films of a suitable lubricant.

When a metallic tube is transported through the reducing die of a draw bench at an elevated speed exceeding 100 meters per minute, proper lubrication of the tube and/or of the die presents serious problems. Even a short-lasting interruption in continuity of the film of lubricant can result in breakage of the moving tube and/or serious damage to the draw bench, particularly to transporting tools with attendant lengthy interruptions in operation and losses in output.

It was already proposed to feed a lubricant between a moving elongated metallic workpiece and the diameter-reducing device of a draw bench at an elevated pressure which suffices to insure that the external surface of the moving workpiece is separated from the reducing device by a continuous layer of lubricant. Wire drawing machines are equipped with apparatus which supply lubricant at a pressure high enough to prevent any mechanical contact between the rapidly moving blank and the component parts of the machine. Thus, the reduction of wire diameter in such machines is attributable mainly to hydrostatic pressure and only indirectly to action of the reducing die. The necessary pressurization of lubricant is brought about artificially by resorting to suitable pumps or the like.

Attempts to rely on the same principle in the cold-drawing of metallic tubes have met with little success. The generation of requisite lubricant pressure by means of pumps presents serious problems and contributes significantly to the cost of the cold-drawing operation. Moreover, the admission of highly pressurized lubricant into the region immediately upstream of the reducing die in a draw bench presents additional serious problems. It was further believed that such mode of cold-drawing cannot be resorted to for simultaneous reduction of metallic tubes by a die and by a mandrel which is installed in the interior of the tube in the region of the die. Heretofore known attempts to introduce a highly pressurized lubricant between the external surface of a mandrel and the internal surface of a long metallic tube have met with failure due to leakage of pressurized fluid on its way from a remote pressurizing device toward the mandrel. In addition, the presently known draw benches which operate on the principle of hydrostatic reduction of the diameter and/or wall thickness of a metallic tube are extremely complex and prone to malfunction so that they failed to gain widespread acceptance in the industry.

### SUMMARY OF THE INVENTION

An object of the invention is to provide a novel and improved method of cold-drawing metallic tubes, particularly steel tubes, by relying on the pressure of lubricant which coats the internal and/or external surfaces

of tubular workpieces during transport through the reducing station.

Another object of the invention is to provide a novel and improved method of insuring the formation of and of maintaining a continuous film of lubricant between a rapidly moving metallic tube and internal and/or external diameter- and/or wall thickness-reducing tools in a draw bench.

A further object of the invention is to provide a method which insures satisfactory cold-drawing of metallic tubes at speeds of up to and in excess of 300 meters per minute.

An additional object of the invention is to provide a novel and improved draw bench for cold-drawing of metallic tubes at a high rate of speed and with greatly reduced likelihood of damage to tubes and/or component parts of the draw bench.

Still another object of the invention is to provide a draw bench with novel and improved means for supplying and confining pressurized lubricant at the internal and/or external surfaces of moving metallic tubes.

A further object of the invention is to provide a draw bench wherein the pressurization of lubricant takes place automatically when the draw bench is in use and wherein such pressurization invariably suffices to insure the formation of an uninterrupted film of lubricant between internal and/or external reducing tools and the corresponding surfaces of metallic tubes.

The method of the present invention is utilized for cold-drawing of metallic tubes, especially steel tubes, and comprises the steps of establishing along at least one of the internal and external surfaces of the leading end of a metallic tube a confined tubular layer of pressurized lubricant which tapers slightly toward a circumferentially complete thickness- and/or diameter-reducing surface of a die or mandrel in a draw bench, and conveying the tube lengthwise relative to the reducing surface at an elevated speed with attendant additional pressurization of confined lubricant due in part to frictional engagement between the one surface of the moving tube and the layer of confined lubricant to thereby raise the pressure of confined lubricant to a value at which the one surface of the moving tube remains separated from the reducing surface by a continuous film of lubricant. The initial pressure of lubricant is preferably less than 100 atmospheres superatmospheric pressure, and such pressure is increased to at least ten times the initial pressure when the tube is in motion. The working pressure of lubricant may be in excess of 600 and preferably in excess of 1,000 atmospheres superatmospheric pressure. The tube can be transported lengthwise at a speed of at least 200 and preferably at or in excess of 300 meters per minute.

The improved cold-drawing method can be practiced with seamless tubes or with welded tubes, and the diameter of the one surface of the tube can be reduced from 8-35 millimeters to as low as 3 millimeters. At the same time, the wall thickness of the moving tube can be reduced from 3.5 millimeters or more to less than 1 millimeter.

If desired or necessary, the reduction of the wall thickness and/or diameter of the tube can be effected in two or more passes whereby the tube is being pulled through a first die by transporting mechanism or mechanisms located between the first and second, second and third, etc., dies.

The novel features which are considered as characteristic of the invention are set forth in particular in the appended claims. The improved draw bench itself, however, both as to its construction and its mode of operation, together with additional features and advantages thereof, will be best understood upon perusal of the following detailed description of certain specific embodiments with reference to the accompanying drawing.

#### BRIEF DESCRIPTION OF THE DRAWING

FIG. 1 is a fragmentary longitudinal sectional view of a draw bench which embodies the invention; and

FIG. 2 is a diagrammatic plan view of a battery of draw benches and transporting devices for metallic tubes.

#### DESCRIPTION OF THE PREFERRED EMBODIMENTS

Referring first to FIG. 1, there is shown a draw bench 2 which is utilized to reduce the internal and external diameters as well as the wall thickness of successive metallic tubes 1. The draw bench 2 includes a frame having a holder 3 for a reducing die 4 which is fixedly but removably received in the holder. The holder 3 further surrounds the front end portion of a confining sleeve 5 which defines with the leading end of a freshly introduced tube 1 a tubular space 12 tapering forwardly toward the die 4 at an angle  $\gamma$  of not more than 3° and preferably about 1.5°. The space 12 surrounds the cylindrical external surface of the leading end of the tube 1 and its length is between 5 and 15 times the external diameter of the tube 1 prior to passage through the die 4. The flange 5a at the forward end of the confining sleeve 5 is pressed against the die by a nut 7 which meshes with the rear end portion of the holder 3. A sealing ring 6 is interposed between the die 4 and flange 5a to prevent escape of lubricant at the front end of the tubular space 12.

The frame of the draw bench 2 further comprises a ring-shaped housing 8 which surrounds the rear end portion of the confining sleeve 5 and is flanked by annular sealing elements 9. A split ring 10 biases the left-hand sealing element 9 against the adjacent end face of the housing 8 with a force which suffices to prevent any appreciable escape of lubricant at both axial ends of the housing. The housing 8 can be slipped off the left-hand end of the sleeve 5 upon removal of the split ring 10.

The housing 8 is provided with an internal annular groove or chamber 8a which communicates with several radial ports 11 of the confining sleeve 5; these ports communicate with the rear portion of the tubular space 12. An inlet opening 13 of the housing 8 communicates with the chamber 8a and is connected with the liquid discharging opening of a pump P which can draw lubricant from a source T. The pump P can be replaced by or provided in addition to an accumulator A. This pump can fill the space 12 with lubricant at a pressure of between 20-100 atmosphere superatmospheric pressure.

The draw bench 2 further comprises a floating mandrel 14a which is located at the front end of an elongated confining member 14 defining with the cylindrical internal surface of the leading end of the tube 1 a second tubular confining space 15 which tapers toward the die 4 at an angle  $\gamma'$  of not more than 3° and prefera-

bly about 1.5°. The axial length of the confining space 15 is preferably at least 5 times and up to 15 times the initial internal diameter of the tube 1. It will be seen that, in the illustrated embodiment, the axial length of the internal confining member 14 equals or approximates the axial length of the sleeve-like external confining member 5.

The cylindrical portion 14a' of the floating mandrel 14a is located in front of a portion 14b having a conical reducing surface which diverges toward the space 15 at an angle  $\beta$  of between 5 and 15°, preferably about 9°. The conical portion 4a of the internal surface of the die 4 diverges toward the space 12 at an angle  $\alpha$  of between 10 and 20°, preferably about 15°. The conical surface of the portion 14b of the mandrel 14a is spaced from and is surrounded by the conical portion 4a of the internal surface of the die 4.

The reference character 16 denotes a supply pipe which furnishes pressurized lubricant from the pump P and/or accumulator A to the rear end of the confining space 15. The initial pressure of lubricant in the confining space 15 is preferably between 20 and 100 atmospheres superatmospheric pressure.

A conduit 17 supplies pressurized lubricant to an axial bore 18 which extends through the confining member 14 and mandrel 14a to admit lubricant to the tubular space 15 of the next draw bench (not shown in FIG. 1) which subjects the once-treated tube 1 to a second cold-drawing treatment.

FIG. 2 illustrates a combination of several draw benches including those numbered 2, 2a, 2b with transporting or pulling devices 30, 30a, 30b located downstream of the corresponding draw benches. Each pulling device comprises a wheel 31 around which the tube 1 forms at least one convolution and which can be driven by a variable-speed electric motor 32. The exact construction of the pulling devices 30, 30a, 30b is disclosed in our copending application Ser. No. 265,969 filed June 26, 1972 and entitled "Multi-pass method and apparatus for cold-drawing of metallic tubes."

The lubricant which is furnished by the conduit 17 of FIG. 1 and passes through the bore 18 of the confining member 14 and mandrel 14a flows through that portion of the once-treated tube 1 which extends between the draw benches 2, 2a and enters the space 15 in the second draw bench 2a. The draw bench 2b may but need not have a mandrel 14a. The conduit 17 may be flexible, either entirely or in part, to insure a satisfactory feed of pressurized lubricant in spite of the fact that the mandrel 14a "floats" in the interior of the tube 1. This conduit 17 can be omitted if the tube 1 is to be subjected to a single cold-drawing treatment.

When the draw bench 2 of FIG. 1 is to be put to use, the leading end of the tube 1 is introduced between the die 4 and mandrel 14a and is convoluted onto the wheel 31 of the pulling device 30. The pump P is thereupon started to draw lubricant from the source T, to pressurize such lubricant, and to introduce it into the confining spaces 12 and 15 at a pressure of between 20 and 100 atmospheres superatmospheric pressure. The motor 32 is started to move the tube 1 lengthwise at a speed of at least 200 and preferably at least 300 meters per minute whereby the pressure of lubricant which is confined in the spaces 12 and 15 automatically rises to at least 600 and preferably 2,000-3,000 atmospheres superatmospheric pressure. Such rise in pressure of lubricant is attributed to friction between the external

and internal surfaces of the tube 1 and the layers of pressurized lubricant in the respective spaces 12 and 15. The highly pressurized lubricant forms uninterrupted films which extend between the external surface of the tube 1 and the internal surface of the die 4 on the one hand, and between the internal surface of the tube 1 and the mandrel 14a on the other hand. The slight taper of spaces 12 and 15, coupled with the high speed of forward movement of the tube 1 and initial pressure of lubricant in the spaces 12 and 15, insures that the reduction in diameter of the tube 1 and the reduction of its wall thickness can be brought about exclusively by hydrodynamic pressure of the lubricant, i.e., without any mechanical contact between the mandrel 14a and/or die 4 and the respective surfaces of the tube 1. The diameter of the tube 1 can be reduced from between 8-35 millimeters to less than 3 millimeters, and the wall thickness of the tube can be reduced from more than 3.5 millimeters to 1.5 millimeters or even less than 1 millimeter. As mentioned above, such reduction in diameter and/or wall thickness can be achieved in a single pass or in two or more passes.

An important advantage of the improved method and draw bench is that the pump P must supply lubricant only prior to and/or during start of a cold-drawing operation and only at a pressure which suffices to insure satisfactory lubrication of the internal and/or external surface of the tube 1. When the operation is started, the pressure of confined lubricant rises automatically to that value which is necessary to insure contactless cold-drawing. Thus, the outlay for the means which subjects the lubricant in the confining space 15 and/or 12 to an initial pressure is only a small fraction of the outlay which would be necessary to artificially maintain the pressure at a value which is needed to insure contactless cold-drawing while the tube is moved lengthwise at the normal speed. The hydrodynamic rise in pressure of lubricant as a result of friction between the moving tube and the stagnant layer or layers of confined lubricant is sufficient to insure the formation of a practically uninterrupted film of lubricant between the reducing surface or surfaces and the respective surface or surfaces of the tube, even if the lubricant is subjected to an initial (artificial) pressure as low as 20 atmospheres superatmospheric pressure.

Another important advantage of the improved method and draw bench is that a continuous film of lubricant can be established and maintained not only between a die and the external surface of a tube but also between the internal surface of the tube and a floating mandrel. The lubricant is sucked and/or pushed into the minute clearances between the reducing surfaces and the corresponding surfaces of the rapidly moving tube whereby the aforescribed length and taper of the spaces 12 and 15 contribute to a rapid and substantial rise in the pressure of confined lubricant to at least ten times the initial pressure. The extent to which the pressure of confined lubricant will rise also depends on the speed of lengthwise movement and surface finish of the tube; these factors influence the friction between the layers of lubricant and the workpiece. The actual reduction in the wall thickness and diameter of the tube is effected by the highly pressurized lubricant in the region of conical surfaces on the mandrel 14a and in the die 4. When the draw bench is in use, there develops an equilibrium between the necessary diameter- and wall thickness-reducing pressure and the maximum

achievable pressure of lubricant; therefore, the reducing action is practically independent of the initial wall thickness and diameter as well as quality of the material of the tube, as long as the length of the spaces 12, 15, their taper toward the die and the finish of surfaces on the tube remain unchanged and the tube is transported at a sufficiently high speed (a feature which is evidently desirable in cold-drawing of metallic tubes).

The taper of the spaces 12 and 15 will be selected in dependency on the roughness or smoothness of the corresponding surfaces of the tube as well as on the speed at which the tube is transported through the die 4. As mentioned above, the moving tube can increase the initial pressure of lubricant to at least 600 and preferably at least 1,000 atmospheres superatmospheric pressure, and the speed of the tube 1 is preferably at least 200 and most preferably about 300 meters per minute, i.e., a speed which is much higher than in presently known draw benches.

The improved method and apparatus can be utilized for treatment of seamless metallic tubes as well as for treatment of welded tubes. The initial diameter of the tubes is preferably in the range of 8-35 millimeters and the initial wall thickness is less than 3.5 millimeters or even less than 1.5 millimeters. As mentioned above, the wall thickness of the tubes can be reduced to less than 1 millimeter and their diameter to less than 3 millimeters, especially by utilizing a battery of two or more draw benches and interposed transporting or pulling devices.

Without further analysis, the foregoing will so fully reveal the gist of the present invention that others can, by applying current knowledge, readily adapt it for various applications without omitting features which fairly constitute essential characteristics of the generic and specific aspects of our contribution to the art and, therefore, such adaptations should and are intended to be comprehended within the meaning and range of equivalence of the claims.

We claim:

1. A method of cold-drawing metallic tubes, particularly steel tubes, which comprises establishing along the internal and external surfaces of the leading end of a tube confined layers of pressurized lubricant which respectively taper slightly forwardly toward a circumferentially complete thickness-reducing external surface of a floating mandrel and toward a circumferentially complete thickness-reducing internal surface of a reducing die; and conveying the tube lengthwise relative to the reducing surfaces at an elevated speed with attendant additional substantial pressurization of lubricant due to frictional engagement between the layers of lubricant and said internal and external surfaces to thereby raise the pressure of confined lubricant to a value at which said internal and external surfaces of the moving tube remain separated from the respective reducing surfaces by continuous films of lubricant.

2. A method as defined in claim 1, wherein the length of one of said confined layers, as considered in the direction of movement of the tube, equals or approximates the length of the other of said layers.

3. A method as defined in claim 1, wherein the initial pressure of lubricant forming said layers is less than 100 atmospheres superatmospheric pressure and said value is at least ten times said initial pressure.

4. A method as defined in claim 3, wherein said value is at least 600 atmospheres superatmospheric pressure.

5. A method as defined in claim 1, wherein said conveying step comprises moving the tube at a speed of at least 200 meters per minute.

6. A method as defined in claim 5 wherein said speed is in excess of 300 meters per minute.

7. A method as defined in claim 1, wherein said tube is a seamless tube.

8. A method as defined in claim 1, wherein said tube is a welded tube.

9. A method as defined in claim 1, wherein the initial diameter of said external surface of the tube is between 8 and 35 millimeters.

10. A method as defined in claim 1, wherein the initial wall thickness of the tube is less than 3.5 millimeters.

11. A method as defined in claim 10, wherein the initial wall thickness of the tube is less than 1.5 millimeters.

12. A method as defined in claim 1, wherein said conveying step comprises pulling the tube at at least one point located downstream of said thickness-reducing surfaces, and further comprising the step of subjecting the once drawn tube to at least one additional cold-drawing operation with attendant additional reduction in wall thickness and external diameter of the tube.

13. A method as defined in claim 12, wherein the final wall thickness of the tube at most equals or slightly exceeds 1 millimeter.

14. A method as defined in claim 12, wherein the final outer diameter of the tube approximates 3 millimeters.

15. In a draw bench for cold-drawing of metallic tubes, particularly steel tubes, a combination comprising a reducing die; first confining means located upstream of said die and defining with the external surface of a tube which extends into said die a first tubular space tapering toward said die; a mandrel disposed within the tube in the interior of said die; second confining means disposed behind said mandrel and defining with the internal surface of the tube a second tubular space which tapers toward said mandrel; means for introducing into said tubular spaces a lubricant at an elevated pressure so that such lubricant completely fills said tubular spaces; and conveying means for moving the tube lengthwise at an elevated speed with attendant additional substantial pressurization of confined lubricant in said tubular spaces due to frictional engagement between the lubricant and the external and internal surfaces of the moving tube to thereby raise the pressure of lubricant in said tubular spaces to a value at which said external and internal surfaces of the moving tube respectively remain separated from said die and from said mandrel by continuous films of lubricant.

16. A combination as defined in claim 15, wherein the taper of said spaces is in the range of at most about 55

3°.

17. A combination as defined in claim 16, wherein the taper of said spaces is at most 1.5°.

18. A combination as defined in claim 15, wherein the axial length of said first space is between 5 and 15 times its internal diameter.

19. A combination as defined in claim 15, wherein said die has an internal surface including a conical portion diverging toward said first space at an angle of between 10 and 20°.

20. A combination as defined in claim 15, wherein the taper of said second space is in the range of at most 3°.

21. A combination as defined in claim 20, wherein the taper of said second space is at most 1.5°.

22. A combination as defined in claim 15, wherein the axial length of said second space is between 5 and 15 times its external diameter.

23. A combination as defined in claim 15, wherein said mandrel has an external surface including a conical portion which diverges toward said second space at an angle of between 5 and 15°.

24. A combination as defined in claim 15, wherein the length of said first tubular space equals or approximates the length of said second tubular space.

25. In an apparatus for cold-drawing of metallic tubes, particularly steel tubes, a combination comprising a battery of at least two draw benches each having a reducing die, first confining means located upstream of the die and defining with the external surface of a tube which extends into said die a tubular space tapering toward the die, a floating mandrel disposed within the tube in the interior of the die, second confining means disposed behind said mandrel and defining with the internal surface of the tube a second tubular space which tapers toward said mandrel, and means for introducing into said tubular spaces a lubricant at an elevated pressure so that the lubricant completely fills said spaces; first conveying means located downstream of that one of said draw benches through which a tube passes prior to entering the other of said draw benches; and second conveying means located downstream of said other draw bench, said first and second conveying means being arranged to move a tube lengthwise at an elevated speed with attendant additional substantial pressurization of confined lubricant in said spaces of said draw benches due to frictional engagement between the lubricant and the external and internal surfaces of the moving tube to thereby raise the pressure of lubricant in said spaces to a value at which said external and internal surfaces of the moving tube respectively remain spaced from said dies and from said mandrels by continuous films of lubricant.

\* \* \* \* \*